

## UNITED STATES PATENT OFFICE

2,153,496

## EXTREME PRESSURE LUBRICANT

Henry G. Berger, Woodbury, Robert C. Moran,  
Wenonah, and Francis M. Seger, Pitman,  
N. J., assignors to Socony-Vacuum Oil Com-  
pany, Incorporated, New York, N. Y., a cor-  
poration of New York

No Drawing. Application April 8, 1938,  
Serial No. 240,910

13 Claims. (Cl. 87—9)

This invention has to do with the art of extreme pressure lubrication and is more particularly concerned with the development of new and improved lubricant compositions which possess the property of maintaining an effective lubricant film between engaged surfaces under high load pressures and high rubbing speeds.

As is well known to those familiar with the art, automobile design over the past several years has involved the use of smaller gears of the worm and hypoid type which operate under extremely high pressure loads and at high rubbing speeds, and as a consequence have required lubricants capable of withstanding pressures much higher than those at which an ordinary hydrocarbon lubricant film of the so-called "thick" type will rupture.

This demand for extreme pressure lubricants has led to the development of various additive ingredients which can be incorporated in a carrying medium such as a mineral oil, which are capable of withstanding, or of yielding a material which will withstand, these extreme pressure conditions. Among the various types of extreme pressure (E. P.) agents which have been proposed are the so-called chemically active type, which possess the property of reacting with the lubricated metal surfaces under the conditions of extreme pressure engagement and forming on such engaged surfaces a "lubricant" film or coating capable of withstanding the extreme pressure loads, thus protecting the engaged metal surfaces against scoring and seizure. The present invention is concerned with the development of improved extreme pressure agents of this general class.

In order that some preliminary indication may be obtained as to the extreme pressure properties of agents or ingredients of this type various laboratory extreme pressure tests have been developed by the automotive industry and the oil industry. Among these tests are the so-called Almen pin test, the S. A. E. test, and the Timken test. These laboratory extreme pressure tests involve the controlled and measured application of load to relatively moving metal surfaces lubricated by the lubricant being tested. Failure of the lubricant is indicated by seizure or scoring of the test pieces.

Although laboratory scale tests of this character offer some indication as to the relative value of extreme pressure agents, they afford little or no indication as to the practicability or impracticability of a particular lubricant composition under actual conditions of commercialization and use. In addition to the property of withstanding the application of extremely high bearing loads

other factors which must be considered in the development of an extreme pressure lubricant are: the tendency of the extreme pressure agent to corrode the containers in which it is stored and the machine parts, such as bearings, housings, and gears, with which the lubricant comes in contact when in use; the tendency of the extreme pressure agent to separate from the carrying medium on standing; the color of the lubricant composition obtained through the use of a particular agent; the tendency of the lubricant composition to develop a cloud or haze; the odor of the additive agent, etc. With the foregoing points in mind it may be observed that there are numerous materials of a chemically active nature which have been proposed as extreme pressure agents and which will satisfy one or more of the laboratory extreme pressure tests. Authorities are in agreement, however, that satisfaction of these tests alone affords no conclusive standard for judging the practical value of an extreme pressure lubricant composition, since many materials which satisfactorily pass such tests are valueless from a practical standpoint because they possess one or more of the undesirable properties enumerated above. It is generally believed, therefore, that actual field and storage tests afford the best means for final evaluation of an extreme pressure agent.

Among the numerous extreme pressure agents of the chemically active type which have been proposed are various metal soaps and compounds containing reactive chlorine, sulfur, and phosphorus. The present invention is concerned with compounds of the type which contain chlorine and sulfur.

Numerous organic materials containing reactive chlorine have been proposed as extreme pressure ingredients, such materials falling into two general classifications, depending upon whether the organic constituent is an aromatic or an aliphatic derivative. In general we have found that in chlorinated compounds of the aromatic type, such as chlorinated naphthalene and chlorinated diphenyl, the chlorine is too firmly bound to the hydrocarbon molecule to have the requisite chemical action upon the bearing metals which will produce the necessary "thin" lubricant film for withstanding the extremely high pressures normally encountered in hypoid gears. Chlorinated aliphatic materials, on the other hand, are too unstable; and while extreme pressure tests on the laboratory machines indicate them to be effective E. P. ingredients, part of the chlorine seems to be very unstable or "highly reactive" so that it is

released under normal conditions of storage and use to form products highly corrosive to containers and metal parts contacted during its use. Chlorinated aliphatic materials as a class are, therefore, not considered commercially usable as extreme pressure ingredients.

Sulfur in the elementary form or in various compounds has also been proposed for extreme pressure lubricants, but here again it is difficult to obtain sulfur in a form which is not unduly corrosive or in a form where it is not so stable as to have little or no practical E. P. value for the high load limits encountered in hypoid gears.

It has long been known that organic compounds containing both sulfur and chlorine such as are obtained by treating mineral oils and fatty oils with sulfur chloride possess the property of increasing the lubricity of mineral lubricating oils, and compounds of this type were among the first considered as possible extreme pressure ingredients. The French patent, No. 683,466 and the corresponding British patent, 454,552, which disclose a multitude of chlorinated organic compounds proposed as extreme pressure ingredients, mention the possibility of using a chlorine compound and a sulfur compound together and also suggest a limited number of compounds containing both sulfur and chlorine. The disclosures are somewhat indefinite as to the composition of these last-mentioned materials, but aryl compounds of sulfur and chlorine appear to be suggested.

As regards compositions or materials containing both sulfur and chlorine, we have found that in general the products obtained by the treatment of a mineral oil or fatty oil with sulfur chloride are too corrosive for practical commercial use. In other words, compounds of this type tend to corrode the containers in which the lubricants are stored and the equipment lubricated. Furthermore, certain of the compounds of this character tend to form highly corrosive sludge on standing. We have also found that as a general proposition the products obtained by chlorinating certain aryl sulfides such as dibenzyl disulfide and the products obtained by chlorinating materials such as dichloroethyl sulfide are too highly reactive for commercial use in that they also break down to form products which attack the containers, the gear housings, etc.

These general observations which we have made as to sulfur-chlorine compounds of the type heretofore proposed have been confirmed by other workers in the field of extreme pressure lubrication. Wolf and Mougey (Proc. A. P. I., 1932, pp. 118-131) have discussed various extreme pressure ingredients, including compounds containing both sulfur and chlorine, and in the addendum to that publication the authors have pointed out that corrosion of steel parts was found to have taken place with the sulfur-chlorine extreme pressure lubricants. In one case the steel parts above the oil level were said to be covered with a heavy layer of iron rust, some of which was washed off by the lubricant and caused rapid bearing wear. The British Patent 431,434 (1935) points out that hydrocarbon extreme pressure lubricants comprised of hydrocarbon base oils containing a sulfur-chlorine compound have objections which have limited or prevented their general use, the chief objection mentioned being the corrosive action of such materials, which causes pitting and rusting of the metal parts and forms oil-insoluble abrasive materials. In a more recently published discussion of chlorine com-

pounds as extreme pressure lubricants (Industrial and Engineering Chemistry, vol. XX, No. 10, pp. 1191-1197) the authors have not mentioned or discussed any proposed extreme pressure ingredients which contain both chlorine and sulfur. It will thus be seen that while organic compounds containing both sulfur and chlorine have received consideration as extreme pressure lubricants and have in fact been shown by the conventional laboratory extreme pressure tests to possess increased load-carrying properties, such compounds have in general been condemned because of their extremely high corrosive action, which makes their storage and use impracticable.

Mere load-carrying ability, therefore, is not the only criterion by which an extreme pressure ingredient can be judged. For commercial use an extreme pressure agent must contain a reactive ingredient or reactive ingredients in a form sufficiently stable to be non-corrosive to the containers and to the machine parts and housings with which it is normally in contact, but at the same time the chemical bond between the reactive ingredient or ingredients and the carrying molecule must be sufficiently unstable to permit a reaction with the metal parts when engaged under extreme pressure to form a "lubricant film" which will carry these high pressure loads. The agents which will satisfactorily meet these requirements are apparently few, and, as stated above, the authorities in this field have generally looked with disfavor on organic compounds containing both sulfur and chlorine because of their highly corrosive action and their tendency to separate on standing.

It is primary object of this invention to provide an extreme pressure ingredient containing both chlorine and sulfur in chemical combination with hydrocarbon material. It is a further object of this invention to produce hydrocarbon materials containing chlorine and sulfur in chemical combinations which possess highly effective extreme pressure lubricant properties and are at the same time devoid of the highly corrosive properties and the tendency to separate normally found present in sulfur-chloride materials which have heretofore been proposed. It is a further object of this invention to provide a method for synthesizing these improved extreme pressure agents.

The new and improved E. P. agents contemplated by this invention may be broadly described as polychlorinated aliphatic hydrocarbon materials in which the more reactive part of the chlorine has been replaced with a sulfur complex. More specifically, the materials contemplated by this invention are polychlorinated aliphatic materials or polychlorinated materials of predominantly aliphatic nature in which a part of the chlorine is replaced by a thiocarbonate group.

We have found that by obtaining a predominantly aliphatic material which contains both chlorine and the thiocarbonate group in chemical combination with the hydrocarbon material, the resulting composition has extremely high load-carrying properties, and extended storage and field tests have demonstrated that it has none of the disadvantages heretofore attributed to sulfur-chlorine-containing compounds.

The preferred procedure which may be followed in synthesizing the E. P. agents contemplated by this invention involves substantial chlorination of an aliphatic compound or a predominantly aliphatic material such as petroleum naphtha, followed by the reaction of the chlorinated ma-

terial with an alkali or alkali earth metal salt of an alkyl thiocarbonic acid in such proportions and under such conditions that only a part of the chlorine (that is, the more reactive chlorine) is replaced by the alkyl thiocarbonate group. The reaction product thus obtained is an aliphatic or predominantly aliphatic hydrocarbon material containing chlorine and thiocarbonate groups in chemical combination with the aliphatic hydrocarbon.

We have found that for the purpose of synthesizing these ingredients the aliphatic material can be chosen from a relatively wide range of aliphatic compounds or hydrocarbon materials which are predominantly aliphatic in nature. The range of aliphatic materials which may be chlorinated as the starting material has been found to extend from polychlorethanes to chlorinated petroleum wax, the former being a compound containing two carbon atoms and the latter being a predominantly aliphatic material corresponding to a compound having substantially twenty carbon atoms. We have found, however, that the extremely short chain compounds represented by polychlorethanes and the extremely long chain compounds represented by petroleum wax are somewhat more difficult to react and are somewhat less efficient in their final composition than hydrocarbons of an intermediate range, and for that reason preference is given to aliphatic materials within the range of from about five to about fifteen carbon atoms, particular preference being given to petroleum naphtha, a hydrocarbon material predominantly aliphatic in nature corresponding to a compound having about ten carbon atoms.

In the chlorination step the aliphatic material is chlorinated to such an extent that the final chlorinated product corresponds to a polychlor compound, and in the case of petroleum naphtha the chlorination is preferably carried to a point at which the product has an average composition corresponding to a tetrachlornaphtha. In general it may be said that chlorination should be carried to the point at which the chlorine content is from about forty per cent to about sixty per cent, although materials of lower and higher chlorine content may be used, depending upon the aliphatic constituent.

The thiocarbonate group which is used to replace a part of the chlorine is, as has been indicated above, derived from an alkali or alkali earth metal salt of a thiocarbonic acid, preferably an alkyl thiocarbonic acid. The thiocarbonate radical may be a mono-, di-, or tri-thiocarbonate, but in general preference is given to the dithiocarbonate (xanthate) compounds, characterized by the divalent group (OCS<sub>2</sub>). The trithiocarbonate type of compounds, characterized by the divalent group (CS<sub>3</sub>) have also been prepared and have been found to form effective extreme pressure agents in combination with the chlorinated aliphatic material, but from the standpoint of odor and cost preference is to products in which the thiocarbonate constituent is a xanthate (divalent OCS<sub>2</sub>) group.

As to the alkyl substituents in the thiocarbonate or xanthate groups which are substituted in the chlorinated aliphatic material, it is preferable that such substituents be derived from aliphatic compounds of relatively low molecular weight. There is no particular advantage to be gained by having a long chain alkyl group in the xanthate or thiocarbonate substituent from the standpoint of solubility, etc., and the lower mo-

lecular weight alkyl groups give a finished product in which the content of chlorine and characterizing divalent thiocarbonate groups (OCS<sub>2</sub>, OCS<sub>2</sub>, or CS<sub>3</sub>) is somewhat more highly concentrated.

As examples of the thiocarbonate or xanthate materials which may be reacted with chlorinated aliphatic materials to provide extreme pressure agents of the type contemplated by this invention, we may use sodium or potassium methyl, ethyl, benzyl, butyl, or amyl xanthates or the corresponding mono- or tri-thiocarbonates.

It is highly important, as stated above, that the proportions of reactants used and the conditions of reaction be controlled so that the final product contains both chlorine and thiocarbonate characterizing groups in chemical combination with the aliphatic hydrocarbon material. The relative amounts of chlorine and sulfur, or, more specifically, of chlorine and thiocarbonate characterizing groups, in the finished product may be varied over a relatively wide range, but in general it may be said that the finished product should preferably be one which contains from about twenty-five to forty per cent chlorine and from about seven to fifteen per cent sulfur. Expressing the sulfur content as the equivalent amount of characterizing thiocarbonate groups present in the product, such preferred products are more accurately identified as containing from about ten per cent to about twenty-two per cent characterizing dithiocarbonate or xanthate (divalent OCS<sub>2</sub>) groups or from about seven per cent to about seventeen per cent characterizing trithiocarbonate (divalent CS<sub>3</sub>) groups. For general purposes it may be said that the characterizing-thiocarbonate-group-content is preferably from about seven per cent to about twenty-two per cent.

The reaction between the chlorinated aliphatic material and the alkali thiocarbonate is preferably carried out in the presence of a relatively low boiling point solvent. For convenience in reaction and purification the solvent is preferably one in which the chlorinated aliphatic material and the reaction product are highly soluble but in which the alkali thiocarbonate and the alkali chloride are of low solubility. As an example of such a solvent we have found acetone to be highly satisfactory, although other solvents, such as methyl ethyl ketone, may be used. Alcohols may also be used as solvents in this reaction. Solvents such as acetone and methyl ethyl ketone are particularly desirable since they permit the reaction to proceed but tend to precipitate residual alkali thiocarbonate and chloride, thus permitting the process to be performed and the product substantially purified all in one step.

The general preferred procedure followed in effecting the replacement of the more highly reactive chlorine in chlorinated aliphatic materials with the thiocarbonate group is to dissolve the chlorinated aliphatic material in the solvent and add the alkali alkyl thiocarbonate in an amount sufficient to give a product having the desired chlorine and sulfur ratio. Under the conditions of reaction which we employ we have prepared materials using from about one-fourth to about twice as much alkali thiocarbonate (xanthate) as chlorinated naphtha. The preferred ratio, however, is to use a weighted amount of alkali thiocarbonate corresponding to from about forty per cent to about seventy per cent of the weight of the chlorinated naphtha used. It will be understood, of course, that these ratios vary with other chlorinated al-

phatic materials, depending upon their hydrocarbon and chlorine content, and should also take into consideration the alkyl substituent which is attached to the characterizing thiocarbonate group.

5 The procedure to be followed in the synthesis of the products contemplated by this invention and the results obtained through the use of such products as extreme pressure agents will be best appreciated from the following examples:

10

*Example I*

As stated above, the preferred products contemplated by this invention are those obtained 15 by replacing a part of the chlorine in chlorinated petroleum naphtha with an alkyl xanthate group. These materials are preferred to others in this general class of materials because of their ease of synthesis, their cost, etc. An exemplary procedure for preparing such a product, which we 20 may term "chlornaphtha-xanthate reaction product" or "xanthochlornaphtha", is as follows:

A chlorinated naphtha was first prepared by 25 chlorinating petroleum naphtha (Stoddard solvent) until it contained about fifty-four per cent by weight of chlorine. 200 parts of the chlor-naphtha were dissolved in about 500 parts of acetone and placed in a reaction vessel heated by a water jacket and equipped with stirrer and reflux condenser. To this solution 120 parts of 30 potassium ethyl xanthate were added and the mixture held at boiling temperature with stirring under reflux for about two hours. The resulting mixture was cooled to room temperature, filtered, 35 and the filtrate subjected to distillation to remove the acetone. After removal of the acetone the product was washed to remove potassium salts and was dried and filtered. The finished reaction product obtained by the foregoing procedure, which for purpose of description herein 40 may be termed "chlornaphtha-xanthate reaction product" or "chlornaphtha-ethyl xanthate reaction product" was a dark brown liquid containing about twelve per cent sulfur, or more specifically about seventeen per cent of the characterizing xanthate (divalent OCS<sub>2</sub>) group, and thirty-seven per cent chlorine.

Variation in xanthate and chlorine content of the reaction product can be obtained by varying 50 the degree of chlorination of the naphtha; by varying the amount of alkali xanthate used; and by varying the hydrocarbon substituent in the alkali xanthate. Thus products of widely varying chlorine and xanthate content are readily 55 possible. In general, as indicated above, we prefer a product containing from about ten per cent to about twenty-two per cent of the characterizing xanthate group and from about twenty-five per cent to about forty per cent of chlorine.

60 In ten per cent concentration in mineral lubricating oil a chlorine-and-xanthate-substituted naphtha obtained as a product from a synthesis such as is described above produces excellent extreme pressure lubricants, passing in a satisfactory manner the usual evaluation tests used in the art. Actual gear tests show the blends to have good extreme pressure properties without any tendency to form sludge and without corrosive action towards the steel parts or towards containers.

70 To show the load-carrying capacity of an extreme pressure agent of the type described in this example, a blend of mineral oil of 80-90 seconds Saybolt Universal viscosity at 210° F. and ten per cent of "chlornaphtha-ethyl xanthate re-

action product" (the reaction product of the foregoing procedure) was subjected to the Almen pin test (described by Wolf and Mougey, Proc. A. P. I., 1932, pp. 118-130) and the S. A. E. test (described Anon. S. A. E. Journal 39, 23-4, 1936) with the following results:

| Almen pin test load limit, lbs. | S. A. E. test load limit, lbs. |                |
|---------------------------------|--------------------------------|----------------|
|                                 | 750 R. P. M.                   | 1,000 R. P. M. |
| 30,000+                         | 580+                           | 470            |
| 30,000+                         | -----                          | 430            |

5

10

15

20

25

30

35

40

45

50

55

60

65

70

75

The oil alone used in the foregoing tests failed in the Almen pin test at a load of 3,000 pounds and showed a load limit of 15 pounds at 1,000 R. P. M. in the S. A. E. test.

In addition to the foregoing extreme pressure tests on laboratory equipment an extreme pressure lubricant of the type described in this example (containing a chlornaphthaethyl-xanthate reaction product of the type described) was subjected to an actual gear test using a hypoid gear loaded at 3500 pounds per linear inch of tooth built up from 0 in thirty-five seconds and held for two hours. Only very slight scratches appeared upon the gear surfaces as contrasted with other so-called extreme pressure lubricants including the lead soap-sulfur compounds, which permitted the gears to score badly under the same test.

At the end of 500 hours in the hypoid gear test with a load of 1100 lb. per lin. in. on the ring gear, a pinion speed of 2500 R. P. M. with intermittent shock loading (on 45 seconds and off 15 seconds), and oil temperature maintained at 180° F., a lead soap-sulfur lubricant showed definite pitting of the gear teeth. After the same severe test, using the reaction product described above in the oil, the gears were not pitted.

To further demonstrate the value of this preferred extreme pressure agent we have conducted an extensive series of field tests using lubricants containing the chlornaphtha-xanthate reaction product as the extreme pressure ingredient in the transmissions and differentials of some thirty-three automobiles operating under varying conditions and in varying localities. At the present time these tests have extended over periods of from about 5000 miles to about 17,000 miles per car, the service of the cars varying from moderate service to extremely severe service. Inspection of the parts so lubricated has been made from time to time, and in all cases the gear condition has been reported either as good or as excellent. In every case the axles were reported as being clean and bright and free from any sludge deposits, and in one instance where our improved lubricant had replaced another so-called extreme pressure lubricant a definite improvement in the cleanliness of the axles was reported. One of the outstanding results obtained through the use of our extreme pressure ingredient was a complete absence of the highly corrosive action on housings and other parts which has been found in and attributed to sulfur-chlorine-containing organic compounds heretofore suggested as extreme pressure agents. These observations are the result of over 800,000 miles of experience in actual service.

Another outstanding feature of the extreme pressure ingredient used in the field tests de-

scribed above was the property of such ingredient of retaining its load-carrying capacity throughout these prolonged service conditions. Samples of the lubricant blend were subjected to the Almen pin test and the S. A. E. test after varying periods of service, and no appreciable loss in load-carrying capacity was observed. In one instance the car had been subjected to 17,474 miles of severe service in high speed operation over gravelled roads, and the lubricant which had been used in this car during such service passed the Almen pin test at 30,000 and gave a load limit of 310 pounds at 1000 R. P. M. on the S. A. E. machine.

In addition to a product of the type described above, which is obtained by the reaction of chlorinated petroleum naphtha and potassium ethyl xanthate and which contains residual chlorine and the characterizing xanthate (divalent  $OCS_2$ ) groups, we have prepared numerous other products of this general type in which:

(a) alkyl xanthates other than the ethyl xanthate group are substituted for the more highly reactive chlorine in chlorinated naphtha;

(b) chlorinated aliphatic materials other than chlorinated naphtha are used as the starting material; and

(c) thiocarbonate groups other than the xanthate group are substituted for the more highly reactive chlorine in chlorinated aliphatic material.

Compounds or materials of these other types are illustrated by the following additional examples:

#### Example II

One hundred parts of chlorinated Stoddard solvent of forty-nine per cent chlorine content) were reacted with fifty-two parts of potassium methyl xanthate, using acetone as a solvent and following the same general procedure described above, except that the mixture was refluxed for one hour. The product obtained, which we may term "chlorinated naphtha-methyl xanthate reaction product", contained 32.45 per cent chlorine and 9.79 per cent sulfur (about fourteen per cent of the characterizing xanthate group). A mineral oil containing ten per cent of this product passed the 30,000 pound load limit in the Almen pin test and showed a load limit of 370 pounds at 755 R. P. M. in the S. A. E. test.

#### Example III

251 parts of chlorinated Stoddard solvent of forty-nine per cent chlorine content) and 120 parts of potassium butyl xanthate were reacted in acetone in the same manner as described in Example II to give a product ("chlorinated naphtha-butyl xanthate reaction product") containing 28.6 per cent chlorine and about thirteen per cent of the characterizing xanthate (divalent  $OCS_2$ ) group. This product in a ten per cent concentration in mineral oil passed the Almen pin test at 30,000 pounds and showed a load limit of 335 pounds at 755 R. P. M. in the S. A. E. test.

#### Example IV

226 parts of chlorinated petroleum wax having a chlorine content of 50.42 per cent were reacted with 200 parts of potassium ethyl xanthate in the presence of acetone with refluxing for two hours to obtain a product ("chlorinated petroleum wax-ethyl xanthate reaction product") containing 37.58 per cent chlorine and about thirteen per cent of the characterizing xanthate group. A ten per cent admixture of this product with mineral oil showed a

load limit of 17,000 pounds in the Almen pin test and of 425 pounds at 755 R. P. M. in the S. A. E. test.

#### Example V

84 parts of tetrachlorethane were reacted with 80 parts of potassium ethyl xanthate in the presence of denatured alcohol as a solvent, the reaction mixture being refluxed for two and one-half hours to obtain a product containing 54.3 per cent chlorine and about 15.9 per cent of the characterizing xanthate group. This product in ten per cent admixture with mineral oil showed a load limit in the Almen pin test of 9,000 pounds and in the S. A. E. test of 230 pounds at 755 R. P. M.

#### Example VI

140 parts by weight of dichloropentane and 70 parts by weight of potassium ethyl xanthate in the presence of acetone as a solvent were refluxed for 1½ hours to yield a "chloropentane-ethyl xanthate reaction product" containing about 27.6 per cent chlorine and about 19.3 per cent of the characterizing xanthate group. A ten per cent blend of this reaction product in a mineral oil of 80-90 seconds S. U. viscosity at 210° F. showed a load limit of 12,000-14,000 pounds in the Almen test and of 345 pounds at 1000 R. P. M. in the S. A. E. test.

#### Example VII

As previously stated, the extreme pressure ingredients contemplated by this invention include products obtained by the chemical substitution of part of the chlorine in a chlorinated aliphatic material with other thiocarbonate groups than the alkyl xanthate (dithiocarbonate) groups discussed in the foregoing examples. To illustrate the preparation of "chlorinated naphtha-alkyl trithiocarbonate reaction products" the following procedure may be used:

Petroleum naphtha (Stoddard solvent) was chlorinated by bubbling chlorine gas therethrough until it contained about fifty-two per cent by weight of chlorine. 225 parts by weight of the chlorinated naphtha were then admixed with about 400 parts of acetone and 100 parts of potassium amyl trithiocarbonate. The mixture was refluxed with stirring on a water bath and heated for about one and a half hours, after which it was cooled and filtered to remove the potassium chloride. The acetone was removed by distillation, after which benzol was added and distilled off to insure removal of water from the product. The resulting product was a bright liquid soluble in oil, and a typical analysis showed a chlorine content of thirty-five per cent and a sulfur content of about ten per cent, or more specifically a trithiocarbonate (divalent  $CS_2$ ) content of about 11.2 per cent. As in the xanthate product, the proportion of chlorine and the proportion of the characterizing trithiocarbonate group in such reaction product may be varied by choice of reactants and proportions used. The nature of the alkyl radical in the alkali alkyl trithiocarbonate may be varied. It will also be understood that in all of the foregoing representative reactions that the alkali metal may be either sodium or potassium.

This trithiocarbonate product ("chlorinated naphtha-amyl trithiocarbonate reaction product"), when blended in ten per cent concentration with a mineral oil of eighty to ninety seconds Saybolt Universal viscosity at 210° F., passed the load limit of 30,000 pounds in the Almen pin test and gave

a load limit of 390 pounds at 1000 R. P. M. in the S. A. E. test.

When the above ten per cent blend of mineral oil was subjected to a heat test by maintaining the blend at a temperature of 300° F. for a period of forty-eight hours with and without the presence of metals, it was found to show a high retention of its original extreme pressure lubricant characteristics. When the oil composition was subjected to the above test in the presence of a copper strip weighing 5.2766 grams, it was found that the copper was not at all pitted and had lost only 0.0180 gram weight. Where a steel pin originally weighing 9.7640 grams was subjected to the same test conditions, the weight lost was only 0.0002 gram, and the surface showed no pitting and no hard coating, showing only a blackening which could be removed easily by rubbing.

#### Example VIII

As a further example illustrating the value of "chlornaphtha-alkyl trithiocarbonate reaction products" for use as extreme pressure ingredients, we have condensed chlorinated petroleum naphtha with a commercial product marketed under the trade name of "Floto". This material, which was used in place of the potassium amyl trithiocarbonate described in Example VI, is made from a mixture of refinery mercaptans and is a mixed sodium trithiocarbonate. The material is predominantly sodium ethyl trithiocarbonate, but the alkyl substituent probably ranges from methyl to amyl. The synthesis of the chlornaphtha trithiocarbonate prepared from this material followed the same procedure outlined above in Example VI, using 100 parts of chlorinated naphtha and 20 parts of "Floto" and 200 parts of acetone. The finished product contained 36.4 per cent chlorine and 7.1 per cent sulfur, or more specifically such product contained 7.9 per cent of the characterizing trithiocarbonate (divalent CS<sub>3</sub>) group.

The lubricating efficiency (load-carrying capacity) tests of the oil blended with the "chlornaphtha-trithiocarbonate reaction product" obtained with "Floto" showed the following results:

| 50 | Concen-<br>tration,<br>percent | Almen pin<br>test load<br>limit, lbs. | S. A. E. at<br>750 R. P. M.<br>load limit,<br>lbs. |
|----|--------------------------------|---------------------------------------|----------------------------------------------------|
|    |                                |                                       | 10<br>5                                            |
|    |                                | 30,000<br>30,000                      | 590+<br>335                                        |

55 The corrosion test for forty-eight hours at 300° F. showed the following results on steel and copper:

| 60          |  | Steel  | Copper |
|-------------|--|--------|--------|
|             |  | Grams  | Grams  |
| Before..... |  | 9.8084 | 5.0777 |
| After.....  |  | 9.8069 | 5.0545 |
| Loss.....   |  | 0.0015 | 0.0232 |

It is will be apparent from the foregoing examples that the products contemplated by this invention may be obtained through the use of various aliphatic hydrocarbon materials and various alkali metal thiocarbonates. From the standpoint of synthesis, cost, and uniformly high results we consider it preferable to use as the starting aliphatic material an aliphatic compound or 70 a mixture of compounds predominantly aliphatic

in nature containing from five to fifteen carbon atoms. Petroleum naphtha, which contains on the average of about ten carbon atoms, is predominantly comprised of aliphatic hydrocarbons, although it may contain some cyclic compounds, but the term "aliphatic material" as it is used herein is intended to include petroleum, naphtha and similar mixed hydrocarbon materials of predominantly aliphatic character. The characterizing thiocarbonate group (divalent XCS<sub>2</sub> in 10 which X is either sulfur or oxygen) in the chlorine-containing reaction products is preferably derived from an alkali alkyl xanthate (the characterizing xanthate group being OCS<sub>2</sub>): but, as shown from the foregoing examples, the trithiocarbonate group (divalent CS<sub>3</sub>) yields products having high load-carrying capacities, which like the xanthate products do not have the highly corrosive tendencies found in sulfur-chlorine-containing organic compounds heretofore proposed as extreme pressure ingredients.

In compounding extreme pressure lubricant compositions with the extreme pressure ingredients described above, mineral lubricating oil is preferred as the carrying medium. However, it is our intention to include within the scope of this invention other "carrying mediums", such as animal oils, vegetable oils, and light mineral oil distillates, in which these E. P. agents may be dispersed with substantial permanence either as true solutions or as colloidal suspensions. The concentration of ingredient used in the suspending or carrying medium may be varied, depending upon the conditions of use, the carrying medium, etc. In general the concentration may be said to range from one per cent to twenty per cent, concentrations of from about five per cent to ten per cent being satisfactory for most purposes where the carrying medium is a mineral lubricating oil.

This application is a continuation in part of 40 our copending applications, Serial No. 123,846, filed February 3, 1937, and Serial No. 159,872, filed August 19, 1937.

We claim:

1. An extreme pressure lubricant composition 45 comprising a major portion of mineral lubricating oil and a minor proportion of a product obtained by chemically substituting a part only of the chlorine in a chlorinated aliphatic material with a thiocarbonate group.

2. An extreme pressure lubricant composition comprising a major portion of mineral lubricating oil and a minor proportion of a product obtained by chemically substituting a part only of the chlorine in a chlorinated aliphatic material with a xanthate group.

3. An extreme pressure lubricant composition comprising a major portion of mineral lubricating oil and a minor proportion of a product obtained by chemically substituting a part only of the chlorine in a chlorinated aliphatic material with a trithiocarbonate group.

4. An extreme pressure lubricant composition comprising a major portion of mineral lubricating oil and a minor proportion of a chlorinated aliphatic hydrocarbon having from about five to about fifteen carbon atoms in which a part only of the chlorine has been chemically substituted with a thiocarbonate group, said product having a chlorine content of from about twenty-five 70 per cent to about forty per cent and a characterizing-thiocarbonate-group content of from about seven per cent to about twenty-two per cent.

5. An extreme pressure lubricant composition

comprising a major portion of mineral lubricating oil and a minor proportion of a chlorinated aliphatic hydrocarbon having from about five to about fifteen carbon atoms in which a part only of the chlorine has been chemically substituted with a xanthate group, said product having a chlorine content of from about twenty-five per cent to about forty per cent and a characterizing-xanthate-group content of from about ten per cent to about twenty-two per cent.

6. An extreme pressure lubricant composition comprising a major portion of mineral lubricating oil and a minor proportion of a chlorinated aliphatic hydrocarbon having from about five to about fifteen carbon atoms in which a part only of the chlorine has been chemically substituted with a trithiocarbonate group, said product having a chlorine content of from about twenty-five per cent to about forty per cent and a characterizing-trithiocarbonate-group content of from about seven per cent to about seventeen per cent.

7. An extreme pressure lubricant composition comprising a major portion of mineral lubricating oil and a minor proportion of a chlorinated petroleum naphtha in which a part only of the chlorine has been chemically substituted with a thiocarbonate group, said product having a chlorine content of from about twenty-five per cent to about forty per cent and a characterizing-thiocarbonate-group content of from about seven per cent to about twenty-two per cent.

8. An extreme pressure lubricant composition comprising a major portion of mineral lubricating oil and a minor proportion of a chlorinated petroleum naphtha in which a part only of the chlorine has been chemically substituted with an alkyl xanthate group, said product having a chlorine content of from about twenty-five per cent to about forty per cent and a characterizing-xanthate-group content of from about ten per cent to about twenty-two per cent.

9. An extreme pressure lubricant composition comprising a major portion of mineral lubricating oil and a minor proportion of a chlorinated petroleum naphtha in which a part only of the chlorine has been chemically substituted with an alkyl trithiocarbonate group, said product having a chlorine content of from about twenty-

five per cent to about forty per cent and a characterizing-trithiocarbonate-group content of from about seven per cent to about seventeen per cent.

10. An extreme pressure lubricant composition comprising a mineral lubricating oil containing as an extreme pressure ingredient from one per cent to twenty per cent of a chlorinated petroleum naphtha in which part of the chlorine has been chemically substituted with an alkyl trithiocarbonate group, said extreme pressure ingredient having a chlorine content of from about twenty-five per cent to about forty per cent and a characterizing-trithiocarbonate-group content of from about seven per cent to about seventeen per cent.

11. An extreme pressure lubricant composition comprising a mineral lubricating oil containing as an extreme pressure ingredient from one per cent to twenty per cent of a chlorinated petroleum naphtha in which part of the chlorine has been chemically substituted with an alkyl xanthate group, said extreme pressure ingredient having a chlorine content of from about twenty-five per cent to about forty per cent and a characterizing-xanthate-group content of from about ten per cent to about twenty-two per cent.

12. An extreme pressure lubricant composition comprising a mineral lubricating oil and a minor proportion of a product obtained by the reaction of chlorinated petroleum naphtha of from about forty per cent to about sixty per cent chlorine content and an alkali alkyl xanthate in the ratio of about fifty to seventy parts by weight of the xanthate to about one hundred parts by weight of the chlorinated naphtha.

13. An extreme pressure lubricant composition comprising a relatively large proportion of an oil and a minor proportion of extreme pressure ingredient dispersed with substantial permanence in said oil, said extreme pressure ingredient comprising a polychlorinated aliphatic material in which a part only of the chlorine has been replaced with an alkyl thiocarbonate group.

HENRY G. BERGER.  
ROBERT C. MORAN.  
FRANCIS M. SEGER.